

# UNITED STATES PATENT OFFICE.

ARTHUR HOWARD HIGGINS, OF LONDON, ENGLAND, ASSIGNOR TO MINERALS  
SEPARATION LIMITED, OF LONDON, ENGLAND.

## TREATMENT OF ORES.

Specification of Letters Patent.

Patented May 29, 1917.

1,227,615.

Application filed November 14, 1913. Serial No. 800,966.

No Drawing.

*To all whom it may concern:*

Be it known that I, ARTHUR HOWARD HIGGINS, a subject of the King of England, residing at London, England, have invented 5 certain new and useful Improvements in the Treatment of Ores, of which the following is a specification.

This invention is for improvements in or relating to the treatment of ores.

10 A number of processes are known in which certain metalliferous constituents of an ore are recovered by methods involving surface tension action, or the selective action of oil, or the formation of a froth, and these processes will hereinafter be referred to as flotation processes. Typical examples of the froth flotation process are described in the prior United States Patent specifications 15 Nos. 835120 granted November 6, 1906 and 20 962678 granted June 28, 1910.

A number of solution or lixiviation processes are also known for the extraction of metals from their ores by the use of chemical agents which dissolve certain metalliferous 25 constituents.

I have discovered that in certain cases these two processes of froth flotation and extraction by solvents can be combined to produce advantageous results. Thus according to this invention, an ore may be agitated with an aqueous liquor which, on the one hand is suitable for bringing about or enhancing a selective separation of certain constituents by flotation and which, on the 30 other hand, brings other constituents into solution.

In the flotation processes above referred to it is customary to add to the aqueous liquor a mineral-frothing agent and also a 40 chemical agent (typified by sulfuric acid) for facilitating the flotation of the metalliferous constituents. According to one embodiment of this invention there is added to the pulp or water in which the agitation 45 takes place, a chemical agent such as ferric chlorid which has the functions (a) of facilitating the flotation of certain metalliferous constituents or parts of the ore, and (b) of dissolving or partially dissolving certain 50 other constituents to be precipitated or removed subsequently. For example, when the ore contains small quantities of copper carbonate this is dissolved and can afterward be precipitated.

55 In previous processes for concentrating

ores by flotation, the flotation has been carried out in water containing various chemical agents, such as alkaline or acid salts, etc., whereby solution of some of the constituents of the ores may be effected to some small extent. In all such processes however, the addition of a chemical agent to the water is not primarily for the purpose of dissolving almost wholly certain constituents of the ore as is the case in the present process, but is employed for various other reasons among which are coating certain metalliferous particles to render them capable of flotation, freeing ores from incrustations and precipitating soluble salts present in the water, or these chemical agents are used in place of the acid generally employed in flotation processes which involve the use of a mineral-frothing agent. The present invention differs from all these known processes in that it comprises a process for the separation of the metalliferous constituents of ores which combines the agitation froth method and extraction of solvents.

The invention will be more fully appreciated by indicating examples of its application. Dealing with an ore containing copper with or without other metals, I have found that by agitating the crushed ore with water containing a mineral-frothing agent (for example an oil) and containing also ferric chlorid, or a mixture of sodium chlorid and ferric sulfate whereby ferric chlorid is produced *in situ*, a certain proportion of the copper, particularly when the mineral is tarnished, is dissolved as copper chlorid, and at the same time a certain proportion of the metalliferous constituents of the ore can be recovered by flotation in the form of a froth. The chemical agent employed may wholly or partially replace the sulfuric acid commonly employed in such flotation processes for facilitating the flotation of the metalliferous constituents.

After removal of the froth and, if desired, after the liquor has been used several times, the solution is removed to a precipitating tank or launder and treated with scrap iron, whereby the copper is precipitated and a solution of iron chlorid is reformed which solution can be used either directly, or preferably after oxidation, in the treatment of further quantities of ore.

This invention affords means for treating complex ores in such a way as to separate

one metalliferous constituent from another. Thus the chemical agent employed may be such as to dissolve more or less completely one particular metal from the ore, while one or more other metals can be recovered by flotation, or the bulk of one metal may be recovered by solution, the bulk of another metal may be recovered by flotation, and the bulk of another metal may be removed in the tailings.

Alternatively, where the ore contains sulfids or metal compounds other than oxidized compounds, the ore may be subjected to a preliminary roasting treatment for the purpose of partially or completely oxidizing certain metalliferous constituents, and thereafter the product may be subjected to the treatment herein above described. For example, an ore containing sulfids and other compounds of copper, lead and zinc, may be roasted to render the copper content soluble in the chemical agent employed. Thereafter the product may be agitated with water containing a mineral-frothing agent and containing also a chemical agent of the kind described for example ferric chlorid; the copper will be dissolved more or less completely, metalliferous constituents such as zinc sulfid can be recovered in the froth, and such products as sulfatized lead compounds will be removed with the tailings.

The chemical agents employed are solutions of salts, as for example ferric chlorid, a convenient strength of solution in the case of the examples given above, being that in which about 1% of the solid ferric chlorid is present.

This invention is not limited to the employment of any particular method of precipitating or removing the metals from solution. Such method may involve the use of precipitates or the removal may be effected by electrolysis by heat, or any of the methods now in use for extracting a metal from its solution.

Among the advantages of this invention may be cited the following:—

Where an ore contains both sulfids and oxids, practically complete metallic recovery may be effected, because the oxidized metals may in the main be dissolved, and the sulfids in the main floated.

Again, in an ore having tarnished surfaces the presence of the chemical agent may effect such a degree of solution as to leave the floatable constituents in good condition for flotation.

What I claim as my invention and desire to secure by Letters Patent is:—

1. A process for the concentration of ores which consists in treating an ore pulp conjointly with a mineral frothing agent for the separation of metalliferous constituents by flotation and with a chemical agent that facilitates the separation of some metallif-

erous constituents by flotation and dissolves other constituents.

2. A process for the concentration of ores which consists in agitating the ore with water containing a mineral-frothing agent and also a chemical agent that facilitates the separation of some metalliferous constituents by flotation and dissolves certain other constituents.

3. A process for the concentration of ores which consists in first roasting the ore and thereafter agitating it with water containing a mineral-frothing agent and also a chemical agent that facilitates the separation of some metalliferous constituents by flotation and dissolves certain other constituents.

4. A process for the concentration of ores which consists in agitating the ore with water containing a mineral-frothing agent and also a chemical agent that facilitates the separation of some metalliferous constituents by flotation and dissolves certain other constituents and thereafter precipitating the dissolved metal from solution in such a manner as to regenerate the chemical agent.

5. A process for the concentration of ores which consists in first roasting the ore and thereafter agitating it with water containing a mineral frothing agent and also a chemical agent that facilitates the separation of some metalliferous constituents by flotation and dissolves certain other constituents and thereafter precipitating the dissolved metal in such a manner as to regenerate the chemical agent.

6. A process for the concentration of ores which consists in treating an ore pulp conjointly with a mineral frothing agent for the separation of metalliferous constituents by flotation and with ferric chlorid, whereby certain constituents of the ore are floated and other constituents are dissolved.

7. A process for the concentration of ores which consists in agitating the ore with water containing a mineral frothing agent and also with ferric chlorid, whereby certain constituents of the ore are floated and other constituents are dissolved.

8. A process for the concentration of ores which consists in first roasting the ore thereafter agitating it with water containing a mineral frothing agent and also ferric chlorid, whereby certain constituents of the ore are floated and other constituents are dissolved.

9. A process for the concentration of ores which consists in treating an ore pulp conjointly with a mineral frothing agent for the separation of metalliferous constituents by flotation and with ferric chlorid produced *in situ* by the reaction of ferric sulfate and sodium chlorid, whereby certain constituents of the ore are floated and other constituents are dissolved.

10. A process for the concentration of ores which consists in agitating the ore with water containing a mineral frothing agent and also ferric chlorid produced *in situ* by the reaction of ferric sulfate and sodium chlorid whereby certain constituents of the ore are floated and other constituents are dissolved.

5 11. A process for the concentration of ores which consists in first roasting the ore and 10 thereafter agitating it with water containing a mineral frothing agent and also ferric

chlorid produced *in situ* by the reaction of ferric sulfate and sodium chlorid whereby certain constituents of the ore are floated and other constituents are dissolved.

15

In testimony whereof I have signed my name to this specification in the presence of two subscribing witnesses.

ARTHUR HOWARD HIGGINS.

Witnesses:

HAROLD CHARLES HANKINS,  
WILLIAM JAMES WALTON.